

## UNITED STATES PATENT OFFICE

2,104,609

## MANUFACTURE OF CERAMIC ARTICLES

Peter de Leeuw, Niagara Falls, N. Y., assignor, by  
mesne assignments, to The Carborundum Com-  
pany, Niagara Falls, N. Y., a corporation of  
Delaware

No Drawing. Application February 9, 1935,  
Serial No. 5,843

4 Claims. (Cl. 51—278)

This invention relates to the production of porous ceramic bodies by the puddled method and particularly to the production of ceramic bonded abrasive articles by the said method.

5 In making porous and/or cellular ceramic articles and particularly abrasive articles by the puddled method two alternative methods are at present employed for controllably increasing the porosity and/or cellularity of the articles when finished.

10 One of these methods comprises the addition of gas evolving substances such as peroxides, carbonates, etc. to the mix and allowing them to decompose while the mass is still in a plastic condition. The gas evolved by the decomposition of the added substances causes the formation of voids and, depending upon the skill with which the mix is handled, these voids will remain until the mix sets sufficiently. The green article is then dried and fired to produce a vitrified article 15 having a cellular structure substantially the same as that of the green article.

20 The other method of producing and controlling the structure of ceramic bodies made by the puddled method comprises adding to the mix combustible particles such as coke, etc. which will be burned out when the article is being fired and will leave voids corresponding in shape and size to those of the combustible particles used.

25 The voids which are formed by the evolution of gas are different in shape than those obtained by the burning out of combustible particles. As a result the articles produced by the two methods have different properties.

30 The evolution of gas produces a structure with a preponderance of discrete voids. The voids are only occasionally interconnected and each one is in the majority of cases completely enclosed in a shell of bond and grain. An article made by such a method might be defined as comprising a plurality of adhering shells of grain and bond, the interior of the said shells interconnecting with adjacent shells only occasionally. On the other hand the method utilizing the combustible particles such as coke produces porous articles having a plurality of irregularly shaped voids which are substantially interconnected. Two articles made by the said methods might be identical in all respects including density but the article made by the burning out of combustible particles would be more permeable than the article made by the evolution of gas.

35 When using the gas method it is difficult if not impossible to obtain an article having a relatively high cellularity made up of relatively

small voids. The size of the voids in an article made by the gas method is affected by the proportion of gas evolving substance in the mix and when a relatively large proportion of such substance is added to the mix to obtain an article 5 having a high cellularity the voids produced in the article are relatively large in size. The tendency of the mix to fall when using the gas method is intensified when a large proportion of gas evolving substance is used in an attempt to obtain 10 an article of great cellularity.

15 Furthermore when the gas method is used a more or less impervious skin or scum is formed over the top of the article while it is being dried. This slows up the rate of drying and causes un- even drying with resultant cracking.

20 When combustible particles such as granulated coke are used in a puddled mix, the coke tends to float to the top of the wheel after the mix is poured into the mold. The coke has a further 25 tendency to ball together in the mix causing the production of undesirably large voids when the wheel is burned.

30 When it is attempted to produce an article of relatively high porosity by the addition of coke to the mix there is a tendency for part of the coke to remain unburned thus defeating the purpose of its addition and resulting in an article of nonuniform porosity.

35 It is an object of the present invention to provide a method of making porous ceramic articles whereby the disadvantages of the prior methods set forth above are obviated, and to produce a ceramic structure having new and unusual characteristics.

40 The present invention comprises the addition to a mix for making a ceramic article by the puddled method, gas evolving substances and comminuted combustible particles, controlling the evolution of gas in the mix before drying to produce a green article having a cellular structure and then burning out the combustible particles during the firing of the article to produce a vitrified article having relatively great porosity.

45 As gas evolving material and combustible material any of the substances previously used alone for this purpose may be used in the combined method of the present invention.

50 In addition the stabilizing agent and catalysts previously used in connection with gas evolving substances to control the rate or degree of evolution of gas may be used in the new method.

55 A great variety of materials and combinations of materials may thus be used in the present invention but the invention will be further de-

scribed in detail in connection with two materials which have been found to be particularly advantageous; that is, coke as the comminuted combustible material and hydrogen peroxide as 5 the gas evolving material.

While the invention is applicable to the production of porous ceramic articles generally, it will be further described with particular reference to the production of a porous abrasive article. The invention may be carried out according to the following example which illustrates one modification of the invention.

*Example*

15 4500 grams of abrasive grain, such as fused alumina, 1500 grams of clay bond and 300 grams of screened coke preferably petroleum coke are mixed together by any suitable means to produce an intimate mixture. The abrasive grain may 20 be of any suitable size and it may be desirable to control the size of the screened coke with reference to the size of the abrasive grain. For example, the abrasive grain of the above mixture may be selected as 80 grit and the coke may be a 25 size which will pass through an 82 mesh screen and be retained by a 109 mesh screen.

16 grams of crystalline sodium pyrophosphate and 1 gram of sodium stannate are dissolved in 2000 cc. of water and added to the dry mix described above. The water solution and the dry ingredients are intimately mixed and then 300 cc. of a 2½% glue solution are added and intimately mixed in. 100 cc. of 4½% hydrogen peroxide solution are then added to the mix and the whole 35 mixed just long enough to incorporate the hydrogen peroxide in the mix uniformly.

The mix or slip is then placed in a suitable mold and allowed to dry. The hydrogen peroxide will decompose before the mix sets and will form 40 a cellular green article.

The dried article is then shaved and cut to a suitable size and placed in a kiln to be burned. During the burning the coke is oxidized to a gas 45 which escapes, resulting in the formation of voids in addition to those formed by the solution of the hydrogen peroxide. The density of a product made in accordance with the above example is about 1.60 and the porosity 54%.

The structure of the article made above, according to the present invention is distinctly 50 different from that of articles made in accordance with previous methods. When a substantial proportion of gas evolving substance such as the hydrogen peroxide is used, the dried green article, 55 before firing, will be a matrix defining a plurality of discrete voids substantially rotund in shape, that is, spherical, oblate, or prolate. When the article is fired the coke will be burned out leaving a plurality of additional voids. These voids will 60 be somewhat irregular in shape following roughly the original shape of the grain of coke which occupied the space. Due to the fact that the grains of coke generally are in contact with other grains of coke throughout the mix, or are adjacent 65 a bubble of gas formed by the evolution of oxygen from the hydrogen peroxide the article will have after the firing thereof a permeable structure in distinction to the somewhat impermeable structure before burning, that is, the voids will substantially all interconnect with at 70 least one adjacent void, with the result that the article will be permeable. The degree of porosity depends upon the proportion of void producing substances used in the mix and the degree of 75 permeability depends roughly upon the propor-

tion of coke used to produce the porosity. The finished article made according to the invention may be said to consist of a matrix of ceramic material which may be a mixture of bond and grain, the matrix defining a plurality of substantially rotund voids interconnected by a plurality of irregular shaped voids. The expression "rotund" is used generally and here specifically to describe shapes partaking of the nature of a fluid bubble which may or may not have been 10 acted upon or constricted by surrounding forces. Such a pore in a ceramic article may be spherical in shape or it may be oblate, prolate or otherwise deformed from the spherical shape but will have relatively smooth walls and the characteristic 15 appearance of a void caused by the expansion of gas.

As stated above, other gas evolving substances than hydrogen peroxide may be used. For example, sodium peroxide, sodium perborate, ammonium persulphate, urea peroxide and other peroxides and per-salts. Instead of coke other granular combustible material may be used such as wood flour, sawdust, seeds and grits obtained from seeds.

25 The hydrogen peroxide concentration may be varied within wide limits. In the manufacture of abrasive articles very good results are still obtainable even if the proportion of the hydrogen peroxide is doubled that used in the example 30 given above. There is no lower limit for the hydrogen peroxide concentration. Small quantities not having any apparent effect on the pore structure may be used for the purpose of deflocculating the mass and to assist in keeping 35 the grain and coke particles in suspension and preventing them from settling out, or balling. The evolution of gas from the decomposition of hydrogen peroxide increases the viscosity of the mix and this further reduces the tendency of the 40 ingredients of the mass to settle out.

The addition of sodium pyrophosphate and sodium stannate to the mix serves to regulate the decomposition of the hydrogen peroxide or other per compounds used to evolve gas and they have 45 the additional action of deflocculating the ingredients of the mix. These ingredients tend to separate the coke into individual particles and thus assist the formation of voids of uniform size. The amount of the coke may be varied up to 50 about 50% or more of the weight of the grain and bond.

The invention has been specifically described with reference to the manufacture of porous abrasive bodies but as stated above the invention 55 may also be applied to the production of other articles, as for example, filter plates, refractory materials such as insulating brick and similar articles. The present invention is of particular use in the manufacture of filter plates having a 60 consistently uniform permeability. By means of the present invention the porosity and pore size can be accurately controlled. The coke particles serve to puncture the film of bond surrounding each void in the cellular structure formed by the 65 gas evolving substances. The permeability of an article can therefore be independently controlled by regulating the absolute and relative amount of combustible particles and gas evolving substance used in the mix.

70 It is thus seen that the two void producing materials added to the mix cooperate to produce beneficial results in the formation of the article and in the article itself which it is not possible to obtain by means of the use of one of them alone. 75

By means of the present invention it is possible to obtain a structure of novel physical characteristics and in addition a structure of lower density than may be obtained by the use of the gas method alone, because in the gas evolving method there is a tendency for the body to fall before it becomes rigid, especially so if much peroxide is added.

Furthermore by means of the present invention it is possible to obtain a puddled article having a high porosity made up of small pores. This is an advantage over the gas method alone because in the latter method a relatively large amount of gas evolving substance is added to the mix in an attempt to obtain a greater porosity or cellularity. The number of voids formed will be substantially the same but the size will be increased to produce the greater cellularity. Without the use of peroxide or other gas evolving substance, the coke has a tendency to float to the top of the puddled wheel thus producing a finished article having a non-uniform distribution of pores. When gas evolving materials are used in the mix together with the coke this difficulty of the separation of the coke does not occur, probably because of the more viscous nature of the gassy mix.

When coke is used in connection with the peroxide method the impervious skin characteristic of the peroxide method does not occur with the result that the surface of the wheel remains pervious enabling it to dry quicker and more evenly.

When the two types of void reducing materials are used in conjunction as in the present invention the tendency of part of the coke to remain unburned when that substance is used alone is obviated. This is apparently because the article is already somewhat cellular when it is put in the kiln for firing due to the previous formation of voids by the action of the gas evolving material. The cellular nature of the green article undoubtedly assists in the complete burning out of the coke during the firing of the article.

By means of the present invention it is possible to produce articles by the puddle method having a controlled pore size and distribution. Articles made by this method are exceptionally uniform in the distribution of the pores. Furthermore by this method it is possible to produce articles having the advantages of the spherical or rotund voids produced by the generation of the gas and the substantial permeability due to the burning out of the combustible particles. By means of the invention it is possible therefore to produce an article having an exceptionally uniform porosity with pores of the desired size and with the desired degree of permeability.

I claim:

1. The method of making a porous abrasive article, which comprises forming a slip comprising abrasive grain and bond, incorporating in the slip granular combustible material and gas evolving material, placing the slip in a mold to permit the gas evolving material to decompose, drying the article and burning it in a kiln to vitrify the bond and burn out the granular combustible material.

2. The method of making a porous abrasive article which comprises forming a slip comprising abrasive grain and bond, incorporating in the mix granulated coke and hydrogen peroxide, placing the mix in a mold to permit the expansion of the article by the evolution of oxygen from the decomposition of the hydrogen peroxide, drying the expanded article and burning it in a kiln to vitrify the bond and burn out the coke particles.

3. The method of making a porous ceramic article which comprises forming a puddling slip containing granular material, a binder therefor, water, granular combustible material and gas-evolving material.

4. The method of making a porous ceramic article which comprises forming a puddling slip containing granular combustible material and gas-evolving material.

PETER DE LEEUW.